

Patented Aug. 13, 1935

2,011,053

# UNITED STATES PATENT OFFICE

2,011,053

## PROCESS FOR PRODUCING OXIDIZED HYDROCARBONS AND PRODUCT THEREOF

Julius Hyman, Chicago, Ill., assignor to Velsicol Corporation, Chicago, Ill., a corporation of Illinois

No Drawing. Application November 18, 1933,  
Serial No. 698,590

6 Claims. (Cl. 260—2)

This invention relates to improvements in the manufacture of oxidized hydrocarbons.

Unsaturated hydrocarbons usually possess the property of absorbing molecular oxygen. The products resulting from such oxidation will vary in consistency, color, reactivity, etc., depending on the nature of the unsaturated hydrocarbons prior to oxidation. Numerous and different types of oxidized hydrocarbons have been reported in the literature.

The present invention has to do with oxidized hydrocarbon mixtures which differ from other such mixtures both in the nature of the starting material and in the oxidized product resulting therefrom.

When petroleum is subjected to vapor phase cracking (that is cracking at temperatures in excess of 1000° F., and at pressures never more than four or five times atmospheric) there results a cracked distillate relatively rich in unsaturated compounds. It has been found that, when the gasoline portion of this distillate is carefully distilled, the first portion of said distillate is colorless. As the distillation proceeds, the color of the distillate becomes progressively a deeper yellow. If, now, the more volatile fractions, (that is, the colorless or very pale colored fractions) are subjected to oxidation by molecular oxygen at temperatures not to exceed 175° F., there results a heavy oxidized polymer of an oleoresinous nature which shows but very little tendency to harden. This oleoresin, whose color is dependent on the temperature of oxidation as well as the color of the starting material, has been found to mix readily with nitrocellulose solutions, and act as an excellent plasticizer for nitrocellulose and other films.

The raw material for the production of the oxidized hydrocarbons of the present invention, consists of the lighter fraction of vapor phase cracked gasoline having a color not yellower than a +16 Saybolt, although the more colorless the raw material, the paler will be the resulting oxidized hydrocarbons, other things being equal.

I have found that the more volatile fractions of the distillate are best suited for the manufacture of this oxidized product. Thus I prefer a distillate which, when distilled in the ordinary Engler apparatus, will distill at least 90% of the starting material before a vapor temperature of 230° F., will have been reached. Different temperatures of vapor phase cracking will produce distillates of differing unsaturation. While, in general, petroleum cracked at about 1200° F., produces highly unsaturated distillates, cracking

temperatures varying from about 1000° F., to about 1400° F., may be employed.

Oxidation should be carried out at as low a temperature as is economically feasible, in order to preserve, insofar as possible, the paleness of the oxidized hydrocarbon. The oxidizing temperature should not exceed about 175° F., although normal atmospheric temperatures are, in general, to be preferred. The oxidation may be speeded up in a number of ways. Increase in temperature and/or pressure will speed up oxidation. The greater the partial pressure of the oxygen used, the more rapid will be the oxidation. The addition to the gasoline fraction of soluble siccative metal compounds, such as soaps of cobalt, manganese, etc., will help greatly to increase the speed of oxidation. It should not be necessary to add more than one-tenth of 1% by weight of the gasoline fraction to be treated of the siccative metal in soap combination, although more or less than this amount may be used if desired. Any combination of the above mentioned methods for hastening oxidation may be employed.

The oxidation described above leaves the major portion of the gasoline unchanged.

After the oxidation has been carried on for a period of time sufficient to produce the desired quantity of oleoresin, the remaining gasoline may be removed either by evaporation or distillation. The latter operation may best be accomplished in a vacuum or under a reduced partial pressure as, for example, by means of a steam distillation. The temperature of the oleoresin during evaporation or distillation should be kept as low as possible in order to insure paleness of color. The temperature of 215° F., should never be exceeded during evaporation or distillation; if possible, the temperature should be kept below 175° F. The recovered gasoline may be used as a motor fuel, or for any other required purpose. As a rule, it will not be necessary to remove all the unoxidized distillate from the oleoresin. Thus, the color of the oleoresin may be further protected.

In order to prevent or retard a further oxidation of the produced oleoresin, there may be mixed with it small quantities of antioxidants, such as hydroquinone, pyrocatechin, para-aminophenol, phenylene diamine, alpha naphthol, alpha naphthylamine, maleic acid, etc. It should never be necessary to add more than 5% the weight of oleoresin as antioxidant, although more may be added if desirable or if compatible. Usually, 1% or less of antioxidant will be found quite sufficient. If desired, the siccative metal may be largely removed from the oleoresin by treatment

with very dilute acids, or by the addition to the oleoresin or oleoresin solution of a water soluble organic acid, such as acetic acid. Such an acid tends to convert the metals present to salts of this acid, which are water soluble and may be removed by washing.

An interesting property of the oxidized resin whose preparation is herein contemplated is that, when heated or baked, it readily turns brown. At 10 the same time, a condensation takes place, with the result that the oleoresin becomes less and less soluble in organic solvents, until finally it assumes what appears to be an insoluble and infusible state. This circumstance suggests the possibility 15 of its use in the preparation of highly resistant baked coatings and impregnants.

I claim as my invention:

1. A process for producing oxidized hydrocarbons which comprises adding to a fraction 20 of gasoline cracked in the vapor phase at temperatures between 1000° and 1400° F. and pressures below 5 atmospheres, at least 90% of such fraction boiling below a temperature of 230° F. and having a color not yellower than +16 Saybolt, a siccative metal drier; subjecting said mixture to the action of molecular oxygen at a temperature below 175° F.; and recovering a heavy 25 oxidized polymer of an oleoresinous nature.

2. A process for producing oxidized hydrocarbons which comprises subjecting a fraction of 30 gasoline cracked in the vapor phase at temperatures between 1000° and 1400° F. and pressures below 5 atmospheres, at least 90% of such fraction boiling below 230° F. and having a color 35 not yellower than +16 Saybolt, to superatmospheric pressure in the presence of molecular oxygen at a temperature below 175° F., and recovering an oxidized polymer of an oleoresinous nature.

3. An oxidized hydrocarbon of oleoresinous nature derived from a fraction of gasoline cracked in the vapor phase at temperatures between 1000° and 1400° F. and pressures below 5 atmospheres, at least 90% of such fraction boiling below 230° F. and having a color not yellower than +16 Saybolt, said fraction having been subjected to the action of molecular oxygen at temperatures below 175° F. 5

4. A plasticizer comprising an oxidized hydrocarbon of oleoresinous nature derived from a fraction of gasoline cracked in the vapor phase at temperatures between 1000° and 1400° F. and pressures below 5 atmospheres, at least 90% of such fraction boiling below 230° F. and having a 10 color not yellower than +16 Saybolt, said fraction having been subjected to the action of molecular oxygen at temperatures below 175° F.

5. A baking varnish comprising an oxidized hydrocarbon of oleoresinous nature derived from 20 a fraction of gasoline cracked in the vapor phase at temperatures between 1000° and 1400° F. and pressures below 5 atmospheres, at least 90% of such fraction boiling below 230° F. and having a 25 color not yellower than +16 Saybolt, said fraction having been subjected to the action of molecular oxygen at temperatures below 175° F.

6. A mixture comprising a relatively small quantity of an antioxidant and an oxidized hydrocarbon of oleoresinous nature derived from a fraction 30 of gasoline cracked in the vapor phase at temperatures between 1000° and 1400° F. and pressures below 5 atmospheres, at least 90% of such fraction boiling below 230° F. and having a 35 color not yellower than +16 Saybolt, said fraction having been subjected to the action of molecular oxygen at temperatures below 175° F.

JULIUS HYMAN.